# EUROPEAN PATENT SPECIFICATION

(11) **EP 1 705 003 B1**
(45) Date of publication and mention of the grant of the patent: **24.10.2007**
(21) Application number: 05102222.6
(22) Date of filing: 21.03.2005
(51) Int. Cl.: B41C 1/10, B41M 5/36

(54) **Processless lithographic printing plates**
Entwicklungsfreie Flachdruckplatten
Plaques d'impression lithographiques sans développement.

(43) Date of publication of application: 27.09.2006
(73) Proprietor: Agfa Graphics N.V., 2640 Mortsel (BE)
(72) Inventor: Groenendaal, Lambertus, Septestraat 27 2640 Mortsel (BE); Van Aert, Hubertus, Septestraat 27 2640 Mortsel (BE); Williamson, Alexander, Septestraat 27 2640 Mortsel (BE); Andriessen, Hieronymus, Septestraat 27 2640 Mortsel (BE)
(74) Representative: Goedeweeck, Rudi

(56) References cited:
- WO-A-02/053627
- US-A1- 2004 023 155

## Description

### FIELD OF THE INVENTION

The present invention relates to a method of lithographic printing and discloses a heat-sensitive printing plate precursor that is suitable for making a lithographic printing plate by direct-to-plate recording.

### BACKGROUND OF THE INVENTION

Lithographic printing presses use a so-called printing master such as a printing plate which is mounted on a cylinder of the printing press. The master carries a lithographic image on its surface and a print is obtained by applying ink to said image and then transferring the ink from the master onto a receiver material, which is typically paper. In conventional, so-called "wet" lithographic printing, ink as well as an aqueous fountain solution (also called dampening liquid) are supplied to the lithographic image which consists of oleophilic (or hydrophobic, i.e. ink-accepting, water-repelling) areas as well as hydrophilic (or oleophobic, i.e. water-accepting, ink-repelling) areas. In so-called driographic printing, the lithographic image consists of ink-accepting and ink-abhesive (ink-repelling) areas and during driographic printing, only ink is supplied to the master.

Printing masters are generally obtained by the image-wise exposure and processing of an imaging material called plate precursor. In addition to the well-known photosensitive, so-called pre-sensitized plates, which are suitable for UV contact exposure through a film mask, also heat-sensitive printing plate precursors have become very popular in the late 1990s. Such thermal materials offer the advantage of daylight stability and are especially used in the so-called computer-to-plate method wherein the plate precursor is directly exposed, i.e. without the use of a film mask. The material is exposed to heat or to infrared light and the generated heat triggers a (physico-)chemical process, such as ablation, polymerization, insolubilization by cross linking of a polymer, heat-induced solubilization, or by particle coagulation of a thermoplastic polymer latex.

The most popular thermal plates form an image by a heat-induced solubility difference in an alkaline developer between exposed and non-exposed areas of the coating. The coating typically comprises an oleophilic binder, e.g. a phenolic resin, of which the rate of dissolution in the developer is either reduced (negative working) or increased (positive working) by the image-wise exposure. During processing, the solubility differential leads to the removal of the non-image (non-printing) areas of the coating, thereby revealing the hydrophilic support, while the image (printing) areas of the coating remain on the support. Typical examples of such plates are described in e.g. EP-A 625728, 823327, 825927, 864420, 894622 and 901902. Negative working embodiments of such thermal materials often require a pre-heat step between exposure and development as described in e.g. EP-A 625,728.

Some of these thermal processes enable plate making without wet processing and are for example based on ablation of one or more layers of the coating. At the exposed areas the surface of an underlying layer is revealed which has a different affinity towards ink or fountain than the surface of the unexposed coating; the image (printing) and non-image or background (non-printing) areas are obtained.

US 5,605,780 discloses a lithographic printing plate comprising an anodized aluminum support and provided thereon an image-forming layer comprising an IR absorbing agent and a cyanoacrylate polymer binder. The image-forming layer is removed by laser-induced thermal ablation whereby the underlying hydrophilic support is revealed.

EP-A 580,393 discloses a lithographic printing plate directly imageable by laser discharge, the plate comprising a topmost first layer and a second layer underlying the first layer wherein the first layer is characterized by efficient absorption of infrared radiation and the first and second layer exhibit different affinities for at least one printing liquid.

EP 1,065,051 discloses a negative-working heat-sensitive material for making lithographic plates comprising in the order given a lithographic base having a hydrophilic surface, an oleophilic imaging layer and a cross-linked hydrophilic upper layer. The heat generated during exposure in the light-sensitive layer removes the hydrophilic upper layer by ablation.

Most ablative plates generate ablation debris which may contaminate the electronics and optics of the exposure device and which needs to be removed from the plate by wiping it with a cleaning solvent, so that ablative plates are often not truly processless. Ablation debris which is deposited onto the plate's surface may also interfere during the printing process and result in for example scumming.

Other thermal processes which enable plate making without wet processing are for example processes based on a heat-induced hydrophilic/ oleophilic conversion of one or more layers of the coating so that at exposed areas a different affinity towards ink or fountain is created than at the surface of the unexposed coating. Such coatings comprise heat-switchable inorganic materials, e.g. zirconia ceramics (US 5,855,173, US 5,839,369 and 5,839,370) or metal oxides (EP 903,223 and US 6,455,222), or organic polymers as described in EP 924,102, WO 92/09934, EP 652,483, US 4,081,572, EP 200,488 and EP 924,065.

WO98/14504 and the doctoral thesis "New Polymers based on the quadruple hydrogen bonding motif" of B.J.B. Folmer, Technische universiteit Eindhoven, 2000, disclose supramolecular polymers containing monomeric units that are bonded in the supramolecular polymer on at least one side via covalent bonds and that can form at least four hydrogen bridges with each other.

WO 02/053626, WO/053627 and US 6,506,536 disclose an imageable element including a thermally sensitive polymer comprising at least one covalently bonded unit and at least one non-covalently bonded unit which includes two or more centered H-bonds. Said thermally sensitive polymer exhibits an increased solubility in an aqueous developer solution upon heating.

US 2004/0023155 discloses an imaging element comprising supramolecular polymers which comprise QHB-modified (quadruple hydrogen bond-modified) polymeric molecules linked via hydrogen bridges. The QHB-modified polymeric molecules comprise two QHB-modified portions A and B, which are linked via a linking group and wherein the A and B portions are selected from a phenolic, acrylic, polyester or polyurethane resin. Upon heating of the imaging element, the QHB-modified polymeric molecules become soluble in an alkaline developer.

### SUMMARY OF THE INVENTION

It is an object of the present invention to provide an alternative printing plate precursor for making a heat-sensitive lithographic printing plate which requires no wet processing step and which can be directly exposed to heat and/or light by means of a laser with low power output.

Surprisingly, it was found that the coating of the heat-sensitive lithographic printing plate precursor according to the method of the present invention, switches from a hydrophilic state to a hydrophobic state or from a hydrophobic state to a hydrophilic state upon exposure to heat. After exposure, the printing plate is ready for printing without the need for further development.

According to the present invention there is provided a method of lithographic printing comprising the steps of
(i) providing a heat-sensitive lithographic printing plate precursor comprising on a support having a hydrophilic surface or which is provided with a hydrophilic layer, a coating comprising a polymer modified with at least two groups which can form four hydrogen bonds, said groups being defined as "quadruple hydrogen bonds" or "QHB" groups;
(ii) exposing said printing plate precursor to heat and/or infrared light whereby the coating switches from a hydrophilic state into a hydrophobic state or from a hydrophobic state into a hydrophilic state, thereby producing a lithographic printing master without an intermediate wet development step;
(iii) supplying ink and/or fountain to said lithographic printing master by means of a lithographic printing press.

According to the present invention there is also provided a printing plate precursor comprising on a support having a hydrophilic surface or which is provided with a hydrophilic layer, a coating comprising a polyether modified with at least two groups which can form four hydrogen bonds, said groups being defined as "quadruple hydrogen bonds" or "QHB" groups.

Preferred embodiments of the present invention are defined in the dependent claims.

### DETAILED DESCRIPTION OF THE INVENTION

The coating of the printing plate precursor according to the method of the present invention comprises a polymer that comprises at least two QHB groups, hereinafter also referred to as a QHB-modified polymer. The QHB groups are attached to the polymer by covalent bonds; these QHB groups may be identical to each other or may be different from each other.

A QHB group is a group capable of forming four hydrogen bonds (i.e. **q**uadruple **h**ydrogen **b**onds or QHB) and can thus be linked via at least four hydrogen bonds to another QHB group. Preferably the QHB group comprises two donor sites and two acceptors sites and the hydrogen bonds are preferably oriented parallel to one another. The QHB group preferably has an essentially flat rigid structure such as for example a flat six-membered ring. A preferred QHB group is an isocytosinyl group.

According to the present invention, a QHB group present on a polymer can associate with a QHB group present on another polymer and a structure with 4-centered hydrogen bonded units is obtained. A schematic presentation of such an association is shown hereafter:

Each QHB group present on the modified polymer can form such a structure and a so-called 'supramolecular polymer' is obtained. Thus the term "supramolecular polymer" in the context of the present invention refers to a polymer which derives it's polymeric properties through a combination of covalent bonds and secondary interactions including hydrogen bonds, more specific four centered hydrogen bonds or quadruple hydrogen bonds (QHB). Such secondary interactions provide high bond strengths and substantially affect the properties of the modified polymers. Between the QHB units other secondary interactions besides hydrogen bonds such as Van der Waals associations, hydrophobic associations, ionic associations or combinations thereof, may also be present. A shematic presentation of a 'supramolecular polymer' is shown hereafter:

The polymer comprising at least two QHB groups is preferably selected from phenolic resins, (meth)acrylic resins, polyester resins, polyether resins, polyurethane resins or mixtures and copolymers thereof.

A QHB-modified polymer can be prepared by reaction of for example, an isocytosine such as a 6-alkyl isocytosine, typically 6-methyl isocytosine, with an isocyanate to produce an isocytosine/isocyanate mono-adduct, i.e. a quadruple hydrogen bonding entity (QHBE). The quadruple hydrogen bonding entity may react with the appropriate polymer to produce the QHB-modified polymer. The 6-methyl isocytosine/isocyanate mono-adduct, a QHBE, is represented by the formula: in which R^{a} is hydrogen, R^{b} is methyl, and Y is an alkylene group derived from a diisocyanate represented by the formula Y(NCO)₂.

Reaction of one mole of the isocytosine with one mole of the diisocyanate produces the QHBE, which will spontaneously dimerize to form a dimeric mono-adduct joined by four thermally reversible hydrogen bonds. The resulting dimeric QHBE has a free isocyanate group on each end, which can react with the appropriate polymer such as an (meth)acrylic polymer, a phenolic polymer, a polyester polymer, a polyether polymer or a polyurethane polymer to produce a QHB-modified polymer such as QHB-modified (meth)acrylic polymer, a QHB- modified phenolic polymer, a QHB-modified polyester polymer, a QHB-modified polyether polymer or a QHB-modified polyurethane polymer.

An alternative method to prepare a QBH-containing polymer is by homopolymerisation of a vinyl monomeric unit containing a QHB group. QBH-containing copolymers can be obtained by copolymerisation of a vinyl monomeric unit containing a QHB group with other vinyl monomeric units.

Carboxyl substituted acrylic polymers may be used as the acrylic polymer. These include, for example, polymers and copolymers of acrylic acid and/or methacrylic acid with, for example, alkyl esters of acrylic acid such as methyl acrylate and ethyl acrylate; alkyl esters of methacrylic acid such as methyl methacrylate and ethyl methacrylate; hydroxyethyl acrylate; hydroxyethyl methacrylate, hydroxypropyl acrylate, hydroxypropyl methacrylate; amides of acrylic acid such as acrylamide and N-methylacrylamide; amides of methacrylic acid such as methacrylamide and N-methylmethacrylamide; acrylonitrile; methacrylonitrile; vinyl chloride; maleic anhydride; itoconic acid; vinylidene chloride; vinyl acetate; vinyl ether; styrene; and N-phenylmaleimide.

In a preferred embodiment the printing plate precursor according to the method of the present invention comprises a polymethacrylate or polyacrylate homopolymer or copolymer which comprises a recurring unit containing a covalently bonded isocytosinyl group in the side chain. The recurring units of the polymethacrylate or polyacrylate homopolymer or copolymer may be represented by the following structures (Figure 1): wherein
R¹ and R² independently represent hydrogen or a hydrocarbon group having up to 12 carbon atoms;
R³ represents hydrogen, an alkyl group, a fluoroalkyl group, an optionally substituted phenyl group, an optionally substituted benzyl group, a pyridyl group, -OR, -COR, -COOR, -OCOR, -NHR, - CONHR, -NHCOR, -NHCOOR, -OCONHR, -NH-CO-NHR or combinations thereof, wherein R represents hydrogen, an optionally substituted alkyl, aryl or a heteroaryl group;
R⁴ and R⁵ independently represent hydrogen, a halogen, an alkoxy or an optionally substituted alkyl, aryl or heteroaryl group;
L¹ represents a divalent linking group;
m/n varies from 100 to 0 and the molecular weight is preferably comprised between 500 and 500000 g/mol.

The substituents optionally present in the phenyl or benzyl groups of R³ may independently be represented by an alkyl group, a halogen such as a chlorine or bromine atom, a carboxylic acid, a sulphonic acid, or a phosphonic acid group, or salts thereof, or a hydroxyl group. The substituents optionally present in the alkyl, aryl or heteroaryl groups of R, R⁴ and R⁵ may independently be represented by a halogen such as a chlorine or bromine atom, a carboxylic acid, a sulphonic acid, or a phosphonic acid group, or salts thereof or a hydroxyl group.

The divalent linking group L¹ represents an alkylene group such as a methylene group, an ethylene group, a propylene group, a butylene group, an isopropylene group; a cycloalkylene group such as cyclohexylene group; an arylene group such as a tolylene group or a heteroarylene group.

More preferrably, the recurring units of the polymethacrylate or polyacrylate homopolymer or copolymer may be represented by the following structures (Figure 2): wherein
R⁶ and R⁷ independently represent hydrogen or a hydrocarbon group having up to 12 carbon atoms;
R⁸ represents hydrogen, an optionally substituted alkyl, aryl or heteroaryl group;
R⁹ and R¹⁰ independently represent hydrogen, a halogen, an alkoxy or an optionally substituted alkyl, aryl or heteroaryl group;
m/n varies from 100 to 0, more preferably between 50 to 0.01, most preferably between 10 and 0.5;; and the molecular weight is preferably comprised between 500 and 500000 g/mol more preferably between 800 and 100000 g/mol and most preferably between 900 and 80000 g/mol.

The substituents optionally present in the alkyl, aryl or heteroaryl groups of R⁸ , R⁹ and R¹⁰ may independently be represented by a halogen such as a chlorine or bromine atom, a carboxylic acid, a sulphonic acid, or a phosphonic acid group, or salts thereof, or a hydroxyl group.

Specific preferred structures of the polymethacrylate or polyacrylate copolymer may be represented by the following compounds I (Figure 3):

### Compound I-1

R¹¹ = R¹² = R¹³ = Me;
m/n = 10;
Mn = 1000-50000 g/mol

### Compound I-2

R¹¹ = R¹² - R¹³ = Me;
m/n = 5.67;
Mn = 1000-50000 g/mol

### Compound I-3

R¹¹ = R¹² = R¹³ = Me;
m/n = 4;
Mn = 1000-50000 g/mol

### Compound 1-4

R¹¹ = R¹² = R¹³ = Me;
m/n = 2.33;
Mn = 1000-50000 g/mol

### Compound I-5

R¹¹ = H;
R¹² = R¹³ = Me;
m/n = 10;
Mn = 1000-50000 g/mol

### Compound I-6

R¹¹ = H;
R¹² = R¹³ = Me;
m/n = 5.67;
Mn = 1000-50000 g/mol

### Compound I-7

R¹¹ = H;
R¹² = R¹³ = Me;
m/n = 4;
Mn = 1000-50000 g/mol

### Compound I-8

R¹¹ = H;
R¹² = R¹³ = Me;
m/n = 2.33;
Mn = 1000-50000 g/mol

Phenolic polymers are typically film-forming polymeric materials that have a multiplicity of phenolic hydroxyl groups either on the polymer backbone or on pendant groups. Novolac resins, resol resins, acrylic resins that contain pendent phenol groups, and polyvinyl phenolic resins are preferred phenolic resins. Other useful phenolic resins include polyvinyl compounds having phenolic hydroxyl groups. Such compounds include, for example, polyhydroxystyrenes and copolymers containing recurring units of a hydroxystyrene, and polymers and copolymers containing recurring units of substituted hydroxystyrenes.

Novolac resins are more preferred. Novolac resins are commercially available and are well known to those skilled in the art. They are typically prepared by the condensation reaction of a phenol, such as phenol, m-cresol, o-cresol, p-cresol, etc, with an aldehyde, such as formaldehyde, paraformaldehyde, acetaldehyde, etc. or a ketone, such as acetone, in the presence of an acid catalyst. The weight average molecular weight is typically about 1,000 to about 15,000 g/mol. Typical novolac resins include, for example, phenol-formaldehyde resins, cresol- formaldehyde resins, phenol-cresol-formaldehyde resins, p-t-butylphenol- formaldehyde resins, and pyrogallol-acetone resins.

Useful polyester polymers may be prepared by reaction of dianhydride compounds with hydroxyl-containing polyester precursors composed of dicarboxylic acid units and glycol units. Useful hydroxyl- containing polyester precursors include, for example, oligoester diols which are the reaction product of a dicarboxylic acid such as succinic acid, adipic acid, azelaic acid, sebacic acid, phthalic acid, isophthalic acid, terephthalic acid, tetrahydrophthalic acid, hexahydrophthalic acid, tetrabromophthalic acid, tetrachlorophthalic acid, 1,4- cyclohexanedicarboxylic acid, maleic acid, fumaric acid, itaconic acid and 5-sodiumsulfoisophthalic acid, with a diol such as ethylene glycol, diethylene glycol, triethylene glycol, polyethylene glycol, 1,2- or 1,3- propanediol, polypropylene glycol, 1,2- or 1,4-butanediol, neopentyl glycol, or 1,6-hexanediol. Useful dianhydrides include, for example, pyromellitic dianhydride, 3,3',4,4'-benzophenone tetracarboxylic dianhydride, 3,3',4,4'-diphenyl tetracarboxylic dianhydride, or 2,3,6,7- naphthalene tetracarboxylic dianhydride.

Useful polyurethane polymers may be prepared by reaction of carboxyl functional diols with diisocyanates. Useful carboxyl functional diols include, for example, dimethylol propionic acid, dihydroxybenzoic acids and the reaction product of a dianhydride such as pyromellitic dianhydride, 3,3',4,4'-benzophenone tetracarboxylic dianhydride, 3,3',4, 4'-diphenyl tetracarboxylic dianhydride, or 2,3,6,7- naphthalene tetracarboxylic dianhydride with a diol such as ethylene glycol, diethylene glycol, triethylene glycol, polyethylene glycol, 1,2- or 1,3- propanediol, polypropylene glycol, 1,2- or 1,4-butanediol, neopentyl glycol, or 1,6-hexanediol.

Useful polyethers are preferably selected from lineair, cyclic or branched polyalkyleneoxides such as for example polyethylene oxide, polypropylene oxide, polybutyleneoxide or mixtures and copolymers thereof. A preferred polyether is a copolymer comprising ethylene oxide and propylene oxide. The polyalkylene oxides preferably include one or more units of the formula -CₙH₂ₙ-O-wherein n is preferably an integer in the range 2 to 5. The moiety - CₙH₂ₙ- may include straight or branched chains. The alkylene moiety may also comprise optional substituents. The molecular weight of the polyether is preferably between 100 g/mol and 5000 g/mol, more preferably between 150 g/mol and 2000 g/mol, most preferably between 150 g/mol and 1500 g/mol.

In another preferred embodiment, the printing plate precursor according to the present invention comprises a QHB-modified polyether. A preferred QHB-modified polyether may be represented by the following structure (Figure 4): wherein
R¹⁴ and R¹⁵ are independently selected from hydrogen, a halogen, a hydroxyl, an alkoxy or an optionally substituted alkyl, aryl or heteroaryl group;
and P¹ is a divalent group comprising a polyether group as described above.

The substituents optionally present in the alkyl, aryl or heteroaryl groups of R¹⁴ and R¹⁵ may independently be represented by a halogen such as a chlorine or bromine atom, a carboxylic acid, a sulphonic acid, or a phosphonic acid group, or salts thereof, or a hydroxyl group.

More preferred QHB-modified polyethers are represented by the following structure (Figure 5): wherein
R¹⁶ and R¹⁷ are independently selected from from hydrogen, a halogen, a hydroxyl, an alkoxy or an optionally substituted alkyl, aryl or heteroaryl group;
L² , L³ , L⁴ and L⁵ each independently represent a divalent linking group;
and P² is a divalent group comprising a polyether group as described above.

The substituents optionally present in the alkyl, aryl or heteroaryl groups of R¹⁶ and R¹⁷ may independently be represented by a halogen such as a chlorine or bromine atom, a carboxylic acid, a sulphonic acid, or a phosphonic acid group, or salts thereof, or a hydroxyl group.

The divalent linking groups L² and L⁵ represents an alkylene group such as a methylene group, an ethylene group, a propylene group, a butylene group, an isopropylene group; a cycloalkylene group such as cyclohexylene group; an arylene group such as a tolylene group, a heteroarylene group.

The divalent linking groups L³ and L⁴ represents an alkylene group such as a methylene group, an ethylene group, a propylene group, a butylene group, an isopropylene group, a cycloalkylene group such as cyclohexylene group, an arylene group such as a tolylene group, a heteroarylene group, -O-, -O-CO-, -NH-, -O-(CH₂)ₖ₋, -(CH₂)ₖ-O-, -(CH₂)ₖ-O-CO-, -O-CO-(CH₂)ₖ-, -(CH₂)ₖ-O-CO-(CH₂)ₗ-, - (CH₂)ₖ-COO-, -CO-O-(CH₂)ₖ-, -(CH₂)ₖ-COO-(CH₂)ₗ-, -(CH₂)ₖ-NH-, -NH-(CH₂)ₖ-, -(CH₂)ₖ-CONH-, -NH-(CH₂)ₖ-O-(CH₂)ₗ-, -(CH₂)ₖ-CO-, -NH-CO-, - NH-CO-O-, -O-CO-NH, -(CH₂)ₖ-CO-NH-, -NH-CO-(CH₂)ₖ-, -NH-CO-NH- or combinations thereof wherein k and 1 are independently an integer greater or equal to 1.

Specific examples of QHB-modified polyethers that are preferred for use in this invention include the following compounds II (Figure 6) :

### Compound II-1

R¹⁸ = R¹⁹ = CH₃
L⁶ = L⁹ = -(CH₂)₆-
L⁷ = L⁸ = -O-
P³ = polyethyleneoxide (Mn = 200 g/mol)

### Compound II-2

R¹⁸ = R¹⁹ = H
L⁶ = L⁹ = -(CH₂)₆-
L⁷ = L⁸ = -O-
P³ = polyethyleneoxide (Mn = 200 g/mol)

### Compound II-3

R¹⁸ = R¹⁹= CH₃
L⁶ = L⁹ = -(CH₂)₆-
L⁷ = L⁸ = -O-
P³ = polyethyleneoxide (Mn = 300 g/mol)

### Compound 11-4

R¹⁸ = R¹⁹= CH₃
L⁶ = L⁹ = -(CH₂)₆-
L⁷ = L⁸ = -O-
P³ = polyethyleneoxide (Mn = 400 g/mol)

### Compound II-5

R¹⁸ = R¹⁹ = CH₃
L⁶ = L⁹ = -(CH₂)₆-
L⁷ = L⁸ = -O-
P³ = polyethyleneoxide (Mn = 900 g/mol)

### Compound II-6

R¹⁸ = R¹⁹= CH₃
L⁶ = L⁹ = -(CH₂)₆-
L⁷ = L⁸ = -O-
P³ = polyethyleneoxide (Mn = 1000 g/mol)

### Compound II-7

R¹⁸ = R¹⁹ = CH₃
L⁶ = L⁹ = -(CH₂)₆-
L⁷ = L⁸ = -NH-
P³ = polyethylene oxide-co-polypropylene oxide
(Mn = 600 g/mol)

### Compound II-8

R¹⁸ = R¹⁹ = CH₃
L⁶ = L⁹ = -(CH₂)6-
L⁷ = L⁸ = -NH-
P³ = polypropylene oxide (Mn = 230 g/mol)

### Compound II-9

R¹⁸ = R¹⁹ = CH₃
L⁶ = L⁹ = 2,4,4-trimethylhexamethylene
L⁷ = L⁸ = -O-
P³ = polyethyleneoxide (Mn = 400 g/mol)

### Compound II-10

R¹⁸ = R¹⁹ = CH₃
L⁶ = L⁹ = -(CH₂)₆-
L⁷ = L⁸ = -O-
P³ = polypropyleneoxide (Mn = 425 g/mol)

Preferrably the printing plate precursor further comprises a monofunctional compound - i.e. a compound comprising one QHB group. More preferably the monofunctional compound is a QHB-modified polyether. The polyether is preferably a polymer comprising straight, branched or cyclic alkylene oxide units such as ethylene oxide or propylene oxide units or mixtures thereof with a molecular weight varying preferably from 100 to 5000 g/mol, more preferably between 150 g/mol and 2000 g/mol and most preferably between 150 g/mol and 1500 g/mol.

Specific monofunctional compounds are represented by the following compounds III (Figure 7) or VI (Figure 8):

### Compound III-1

L¹⁰ = -O-
P⁵ = polyethylene oxide, Mn = 400 g/mol
R²⁰ = OH

### Compound III-2

L¹⁰ = -NH-
P⁵ = polyethylene oxide-co-polypropylene oxide
(Mn = 600 g/mol)
R²⁰ = NH₂

### Compound IV-1

L¹¹ = -(CH₂)₆-
L¹² = -O-
P⁶ = polyethylene oxide (Mn = 400 g/mol)
R²¹ = OH

### Compound IV-2

L¹¹ = -(CH₂)₆-
L¹² = -NH-
P⁶ = polyethylene oxide-co-polypropylene oxide
(Mn = 600 g/mol)
R²¹ = NH₂

According to the present invention there is also provided a printing plate precursor comprising a QHB-modified polyether as described above. Optionally the printing plate precursor may also comprise a monofunctional compound as described above.

The support of the lithographic printing plate precursor has a hydrophilic surface or is provided with a hydrophilic layer. The support may be a sheet-like material such as a plate or it may be a cylindrical element such as a sleeve that can be slid around a print cylinder of a printing press. Preferably, the support is a metal support such as aluminum or stainless steel.

A particularly preferred lithographic support is an electrochemically grained and anodized aluminum support. The anodized aluminum support may be treated to improve the hydrophilic properties of its surface. For example, the aluminum support may be silicated by treating its surface with a sodium silicate solution at elevated temperature, e.g. 95°C. Alternatively, a phosphate treatment may be applied which involves treating the aluminum oxide surface with a phosphate solution that may further contain an inorganic fluoride. Further, the aluminum oxide surface may be rinsed with a citric acid or citrate solution. This treatment may be carried out at room temperature or may be carried out at a slightly elevated temperature of about 30 to 50°C. A further interesting treatment involves rinsing the aluminum oxide surface with a bicarbonate solution. Still further, the aluminum oxide surface may be treated with polyvinylphosphonic acid, polyvinylmethylphosphonic acid, phosphoric acid esters of polyvinyl alcohol, polyvinylsulfonic acid, polyvinylbenzenesulfonic acid, sulfuric acid esters of polyvinyl alcohol, and acetals of polyvinyl alcohols formed by reaction with a sulfonated aliphatic aldehyde. It is further evident that one or more of these post treatments may be carried out alone or in combination. More detailed descriptions of these treatments are given in GB-A- 1 084 070, DE-A- 4 423 140, DE-A- 4 417 907, EP-A- 659 909, EP-A- 537 633, DE-A- 4 001 466, EP-A- 292 801, EP-A-291 760 and US-P- 4 458 005.

According to another embodiment, the support can also be a flexible support, which is provided with a hydrophilic layer, hereinafter called 'base layer'. The flexible support is e.g. paper, plastic film, thin aluminum or a laminate thereof. Preferred examples of plastic film are polyethylene terephthalate film, polyethylene naphthalate film, cellulose acetate film, polystyrene film, polycarbonate film, etc. The plastic film support may be opaque or transparent.

The base layer is preferably a cross-linked hydrophilic layer obtained from a hydrophilic binder cross-linked with a hardening agent such as formaldehyde, glyoxal, polyisocyanate or a hydrolyzed tetra-alkylorthosilicate. The latter is particularly preferred. The thickness of the hydrophilic base layer may vary in the range of 0.2 to 25 µm and is preferably 1 to 10 µm.

Particular examples of suitable hydrophilic base layers for use in accordance with the present invention are disclosed in EP-A-601 240, GB-P- 1 419 512, FR-P- 2 300 354, US-P- 3 971 660, and US-P- 4 284 705.

The coating preferably also contains a compound that absorbs infrared light and converts the absorbed energy into heat. The amount of infrared absorbing agent in the coating is preferably between 0.25 and 25.0 % by weight, more preferably between 0.5 and 20.0 % by weight. In a preferred embodiment, its concentration is at least 6 % by weight, more preferred at least 8 % by weight. The infrared absorbing compound can be present in the image-recording layer and/or an optional other layer. Preferred IR absorbing compounds are dyes such as cyanine, merocyanine, indoaniline, oxonol, pyrilium and squarilium dyes or pigments such as carbon black. Examples of suitable IR absorbers are described in e.g. EP-As 823327, 978376, 1029667, 1053868, 1093934; WO 97/39894 and 00/29214. A preferred compound is the following cyanine dye IR-1: wherein X⁻ is a suitable counter ion such as tosylate, bromide or chloride.

To protect the surface of the coating, in particular from mechanical damage, a protective layer may also optionally be applied. The protective layer generally comprises at least one water-soluble polymeric binder, such as polyvinyl alcohol, polyvinylpyrrolidone, partially hydrolyzed polyvinyl acetates, gelatin, carbohydrates or hydroxyethylcellulose, and can be produced in any known manner such as from an aqueous solution or dispersion which may, if required, contain small amounts, i.e. less than 5% by weight, based on the total weight of the coating solvents for the protective layer, of organic solvents. The thickness of the protective layer can suitably be any amount, advantageously up to 5.0 µm, preferably from 0.05 to 3.0 µm, particularly preferably from 0.10 to 1.0 µm.

The coating may in addition to the image-recording layer also contain one or more additional layer(s). Besides the additional layers already discussed above - i.e. an optional light-absorbing layer comprising one or more compounds that are capable of converting infrared light into heat and/or a protective layer such as e.g. a covering layer which is removed during processing - the coating may further for example comprise an adhesion-improving layer between the image-recording layer and the support.

Optionally, the layer comprising a compound capable of absorbing light or an optional other layer may further contain additional ingredients. For example binders, surfactants such as perfluoro surfactants, silicon or titanium dioxide particles or colorants may be present.

According to the method of the present invention the heat-sensitive printing plate precursor obtained is image-wise exposed directly with heat or indirectly with infrared light, preferably near infrared light. The infrared light is preferably converted into heat by an IR light absorbing compound as discussed above. The printing plate precursor is not sensitive to ambient light so that it can be handled without the need for a safe light environment.

The printing plate precursor can be exposed to infrared light by means of e.g. LEDs or an infrared laser. Preferably, the light used for the exposure is a laser emitting near infrared light having a wavelength in the range from about 700 nm to about 1500 nm, e.g. a semiconductor laser diode, a Nd:YAG or a Nd:YLF laser. The required laser power depends on the sensitivity of the image-recording layer, the pixel dwell time of the laser beam, which is determined by the spot diameter (typical value of modern plate-setters at 1/e² of maximum intensity : 10-25 µm), the scan speed and the resolution of the exposure apparatus (i.e. the number of addressable pixels per unit of linear distance, often expressed in dots per inch or dpi; typical value : 1000-4000 dpi).

Two types of laser-exposure apparatuses are commonly used: internal (ITD) and external drum (XTD) plate-setters. ITD plate-setters for thermal plates are typically characterized by a very high scan speed up to 1500 m/sec and may require a laser power of several Watts. The Agfa Galileo T (trademark of Agfa Gevaert N.V.) is a typical example of a plate-setter using the ITD-technology. XTD plate-setters operate at a lower scan speed typically from 0.1 m/sec to 20 m/sec and have a typical laser-output-power per beam from 20 mW up to 500 mW. The Creo Trendsetter plate-setter family (trademark of Creo) and the Agfa Excalibur plate-setter family (trademark of Agfa Gevaert N.V.) both make use of the XTD-technology.

The known plate-setters can be used as an off-press exposure apparatus, which offers the benefit of reduced press down-time. XTD plate-setter configurations can also be used for on-press exposure, offering the benefit of immediate registration in a multi-color press. More technical details of on-press exposure apparatuses are described in e.g. US 5,174,205 and US 5,163,368.

The exposure step may optionally be followed by a rinsing step and/or a gumming step. The gumming step involves post-treatment of the heat-sensitive printing plate with a gum solution. A gum solution is typically an aqueous liquid that comprises one or more surface protective compounds that are capable of protecting the lithographic image of a heat-sensitive material or printing plate against contamination or damaging. Suitable examples of such compounds are film-forming hydrophilic polymers or surfactants.

The heat-sensitive printing plate is then ready for printing without an additional development step. The exposed plate can be mounted on a conventional, so-called wet offset printing press in which ink and an aqueous dampening liquid are supplied to the material. The non-image areas hold the dampening water and the image areas withhold the ink.

Another suitable printing method uses so-called single-fluid ink without a dampening liquid. Suitable single-fluid inks have been described in US 4,045,232; US 4,981,517 and US 6,140,392. In a most preferred embodiment, the single-fluid ink comprises an ink phase, also called the hydrophobic or oleophilic phase, and a polyol phase as described in WO 00/32705.

Alternatively, the printing plate is first mounted on the printing cylinder of the printing press and then image-wise exposed directly on the press by means of an integrated image-recording device. Subsequent to exposure, the plate is ready for printing.

The printing plate precursor according to the present invention comprising the QHB-modified polyether may be exposed and optionally post-treated with a gum solution or water (both steps as described in detail above) whereby a printing master is obtained. The printing step can be carried out as described above.

### EXAMPLES

### PREPARATION OF THE COMPOUNDS.

The chemicals used in the synthesis described below are commercially available. The preparation method of 4-cyano-4-[(phenylthioxomethyl)thio] pentanoic acid is described in S.H. Thang, B. Y. K. Chong, R. T. A. Mayadunne, G. Moad, E. Rizzardo, Tet. Lett., 1999, 40, 2435.

### 1.1. Preparation of compounds I-3, I-6 and I-7.

### Preparation of 2-methyl-, 2-[[[(1,4-dihydro-6-methyl-4-oxo-2-pyrimidinyl)amino]carbonyl]amino]ethyl methacrylate.

5.0g 2-Amino-4-hydroxy-6-methylpyrimidine was dissolved in 65 ml dimethylsulphoxide by heating to 170 °C. To the solution 6.8g isocyanatoethylmethacrylate was added. The mixture was stirred for 20 minutes and then cooled in an ice-bath. The resultant precipitate was diluted with acetone and then filtered to give the desired product. Yield = 7.0g, 78%.

### Preparation of Compound I-7.

Into a half litre three-necked flask 1.52g acrylic acid, 1.48g 2-methyl-, 2-[[[(1,4-dihydro-6-methyl-4-oxo-2-pyrimidinyl)amino]carbonyl]amino]ethyl methacrylate and 25ml 1-methoxy-2-propanol were added. Subsequently, 0.074g 4-cyano-4-[(phenylthioxomethyl)thio] pentanoic acid and 0.067g 4,4'-Azobis(4-cyanovaleric acid) were added to this solution. The solution was then degassed by bubbling nitrogen through for 60 minutes. The polymerisation was started by warming the mixture up to 85 °C and was kept at this temperature for 5 hours. The mixture was then allowed to cool down. The precipitate was filtered off, washed with methylene chloride and then dried. Yield = 2.19g, 73%, Mn = 11310 g/mol.

### Preparation of Compound I-3.

1-3 was made by the same method as compound I-7, with the following amounts of starting materials. Methacrylic acid (2.21g), 2-[[[(1,4-dihydro-6-methyl-4-oxo-2-pyrimidinyl)amino]carbonyl]amino]ethyl methacrylate (1.79g), methoxypropanol (40 mL), 4-cyano-4-[(phenylthioxomethyl)thio] pentanoic acid (0.081g), 4,4'-Azobis(4-cyanovaleric acid) (0.081g). Yield = 3.0g, 73%, Mn = 11530 g/mol.

### Preparation of Compound I-6.

To a mixture of 2.96g acrylic acid and 2.04g 2-[[[(1,4-dihydro-6-methyl-4-oxo-2-pyrimidinyl)amino]carbonyl]amino]ethyl methacrylate, 0.11g dimethyl-2,2'-azobisisobutyrat, 0.11g 2-4-diphenyl-4-methyl-1-pentene and 44.77g isopropanol were added. The mixture was degassed for 3 minutes and then heated at 90 °C for 6 hours under a stream of nitrogen. The product was collected by filtration, washed with acetone and dried. Yield = 2.9g, 58%, Mn = 12400 g/mol.

### 1.2. Preparation of compounds II-3, II-4/IV-1 and II-7.

### Preparation of N-(1,4-dihydro-6-methyl-4-oxo-2-pyrimidinyl)-N'-(6-isocyanatohexyl)urea.

Based on procedure descibed in doctoral thesis "New Polymers based on the quadruple hydrogen bonding motif" of B.J.B. Folmer, Technische universiteit Eindhoven, 2000, page 95.

72.0g Hexamethylene diisocyanate was added to a 100ml flask and heated under a nitrogen atmosphere to 80 °C. To this mixture 12.0g 2-Amino-4-hydroxy-6-methylpyrimidine was added. The mixture was then warmed to 100 °C and stirred for 20 hours. The mixture was then allowed to cool and the precipitate isolated by filtration and washing with n-hexane. Yield = 27.3g, 97%.

### Preparation of compound II-3.

The synthetic method is based on the method described in the following reference: H. M. Keizer, R. van Kessel, R. P. Sijbesma, E. W. Meijer, Polymer, 2003, 44, 5505.

A solution of 2.55g polyethyleneglycol (Mn = 300g/mol) and 300 ml toluene was warmed to 60 °C and then 5.0g N-(1,4-dihydro-6-methyl-4-oxo-2-pyrimidinyl)-N'-(6-isocyanatohexyl)urea was added together with 5 drops of dibutyltin dilaurate. The mixture was refluxed with stirring for 2.5 hours at 113°C, allowed to cool to 105 °C, and then a further 1.05g of then N-(1,4-dihydro-6-methyl-4-oxo-2-pyrimidinyl)-N'-(6-isocyanatohexyl)urea was added. Subsequently the mixture was refluxed for a period of 5.5 hours. The mixture was allowed to cool to 105 °C and a further 0.12g of then N-(1,4-dihydro-6-methyl-4-oxo-2-pyrimidinyl)-N'-(6-isocyanatohexyl)urea was added. The mixture was refluxed for a further 6.5 hours and then allowed to cool to room temperature. The solvent was removed in vacuum and the solid residue extracted with warm methoxypropanol. The solvent was removed from the extract and the resultant solid washed with ethyl acetate. Yield = 4.5 g, 60%.

### Preparation of mixture of Compound II-4 and IV-1.

To a solution containing 6.0g N-(1,4-dihydro-6-methyl-4-oxo-2-pyrimidinyl)-N'-(6-isocyanatohexyl)urea and 4.0g polyethylene glycol (Mn = 400g/mol) in 400 ml methylene chloride and 40 ml dimethylsulphoxide were added 5 drops of dibutyltin laurate. The mixture was then refluxed for 24 hours. The mixture was allowed to cool to room temperature and the precipitate removed by filtration. The filtrate was then reduced under vacuum to a solid which was then treated with ethyl acetate and n-hexane to produce a solid which was isolated by filtration. Yield = 2.7g.

### Preparation of compound II-7.

To a 500 ml flask 5.0 g N-(1,4-dihydro-6-methyl-4-oxo-2-pyrimidinyl)-N'-(6-isocyanatohexyl)urea, 5.1 g Jeffamine ED-600 (tradename of Huntsman Corporation, CASRN 65605-36-9), 40 ml methylene chloride, 40 ml dimethylsulphoxide and 5 drops of dibutyl tin dilaurate were added. The mixture was refluxed with stirring for 24 hours. Addition of 500 ml methanol followed by filtration and removal of solvent from the filtrate gave the required product which was washed with ethyl acetate and dried. Yield = 9.2 g, 90%.

### PREPARATION OF THE COATING SOLUTIONS.

### Invention Example 1.

A mixture of Compound II-4 and compound VI-1 was added to DMSO and the mixture was warmed to about 80 °C while stirring until a clear solution was obtained. IR-2 was added to this solution (Table 1) .

### Invention Examples 2, 3 and 4.

Compound Type I-3, I-6 or I-7 was added to a mixture of THF, water and triethylamine. To this solution IR-1 was added (Table 1).

**Table 1: Compositions of the coating solutions.**

| Ingredients | Invention Example 1 | Invention Example 2 | Invention Example 3 | Invention Example 4 |
|---|---|---|---|---|
| Compound II-4 g | 1.31 | - | - | - |
| Compound VI-1 g | 0.34 | - | - | - |
| Compound I-3 g | - | 0.5 | - | - |
| Compound I-6 g | - | - | 0.5 | - |
| Compound I-7 g | - | - | - | 0.5 |
| Tetrahydrofuran ml | - | 5.94 | 5.94 | 5.94 |
| Dimethylsulfoxide ml | 48.6 | - | - | - |
| Triethylamine ml | | 1.25 | 1.25 | 1.25 |
| Water ml | | 5.94 | 5.94 | 5.94 |
| IR-1 (1) ml | - | 1.88 | 1.88 | 1.88 |
| IR-2 (2) ml | 0.25 | - | - | - |

| | | | | |
|---|---|---|---|---|
| (1): 2% dispersion in water, infrared absorbing dye IR-1 has the following structure: (2) : 2% dispersion in water, infrared absorbing dye IR-2 has the following structure: | | | | |

### PREPARATION OF THE PRINTING PLATES.

The coating solutions were coated with a bar-coater (thickness of layer 30 microns) onto an anodised aluminium plate at 40 °C and then dried for 10 minutes at 40 °C (Invention Examples 2, 3 and 4) and at 95 °C (Invention Example 1).

### PRINT RESULTS.

The plates were then exposed using an 830 nm IR laser (Isomet Diode) with the energy densities indicated in the Table 3 below.

**Table 3: Applied Energy Densities.**

| Power mW | Drumspeed m/s | Energy density mJ/cm² |
|---|---|---|
| 4 | 200 | 714 |
| 4 | 140 | 500 |
| 4 | 100 | 357 |
| 8 | 200 | 357 |
| 8 | 100 | 179 |
| 8 | 60 | 107 |

The plate was then ready for printing. The printing test was performed on an off-set printing press GTO 46 (available from Heidelberger Druckmaschinen AG) using K + E Novavit 800 Skinnex ink (trademark of BASF Drucksysteme GmbH) and Agfa Prima FS101 fountain solution (trademark of Agfa). Minimum sensitivity is defined as the lowest energy at which a clear image is visible after 250 prints (Table 4).

**Table 4: print results.**

| | Image Type | Minimum |
|---|---|---|
| | | sensitivity* |
| Invention Example 1 | Positive | 179 mJ/cm² |
| Invention Example 2 | Negative | 714 mJ/cm² |
| Invention Example 3 | Negative | 500 mJ/cm² |
| Invention Example 4 | Negative | 357 mJ/cm² |

| | | |
|---|---|---|
| * the lowest energy at which a clear image is visible after 250 prints. | | |

The results in Table 4 show that Invention Example 1 results in a positive-working printing plate and that with Invention Examples 2, 3 and 4 a negative working printing plate is obtained. The highest sensitivity is obtained for the positive working printing plate of Invention Example 1.

## Claims

1. A method of lithographic printing comprising the steps of
(i) providing a heat-sensitive lithographic printing plate precursor comprising on a support having a hydrophilic surface or which is provided with a hydrophilic layer, a coating comprising a polymer modified with at least two groups which can form four hydrogen bonds, said groups being defined as "quadruple hydrogen bonds" or "QHB" groups;
(ii) exposing said printing plate precursor to heat and/or infrared light whereby the coating switches from a hydrophilic state into a hydrophobic state or from a hydrophobic state into a hydrophilic state, thereby producing a lithographic printing master without an intermediate wet development step;
(iii) supplying ink and/or fountain to said lithographic printing master by means of a lithographic printing press.

2. A method according to claim 1 wherein at least one of the QHB groups is an isocytosinyl group.

3. A method according to claims 1 or 2 wherein the polymer is selected from QHB-modified phenolic resins, QHB-modified poly(meth)acrylates, QHB-modified polyesters, QHB-modified polyethers, QHB-modified polyurethanes or mixtures and copolymers thereof.

4. A method according to claim 3 wherein the polymer is a QHB-modified polyether.

5. A method according to claim 4 wherein the molecular weight of the QHB-modified polyether is comprised between 100 g/mol and 5000 g/mol.

6. A method according to any of claims 4 or 5 wherein the QHB-modified polyether is selected from QHB-modified polyethylene oxide or QHB-modified polypropylene oxide or mixtures and copolymers thereof.

7. A method according to claim 3 wherein the polymer is a QHB-modified (meth)acrylate homopolymer or copolymer comprising a recurring unit comprising an isocytosinyl group in the side chain.

8. A method according to claim 7 wherein the QHB-modified (meth)acrylate homopolymer or copolymer has a molecular weight ranging from 500 to 500000 g/mol.

9. A printing plate precursor comprising on a support having a hydrophilic surface or which is provided with a hydrophilic layer, a coating comprising a polyether modified with at least two groups which can form four hydrogen bonds, said groups being defined as "quadruple hydrogen bonds" or "QHB" groups.

10. A printing plate precursor according to claim 9 wherein the QHB group is an isocytosinyl group.

11. A printing plate precursor according to claims 9 or 10 wherein the molecular weight of the modified polyether is comprised between 100 g/mol and 5000 g/mol.

12. A printing plate precursor according to claim 11 wherein the modified polyether is selected from QHB-modified polyethylene oxide or QHB-modified polypropylene oxide or mixtures thereof.

## Patentansprüche

1. Ein durch die folgenden Schritte **gekennzeichnet**es lithografisches Druckverfahren :
(i) Bereitstellen einer wärmeempfindlichen lithografischen Druckplattenvorstufe, die auf einem Träger, der eine hydrophile Oberfläche aufweist oder mit einer hydrophilen Schicht versehen ist, eine Beschichtung mit einem Polymer enthält, das mit zumindest zwei Gruppen, die vier Wasserstoffbrückenbindungen bilden können, modifiziert ist, wobei die Gruppen als "vierfache Wasserstoffbrückenbindungen" oder "VWB"-Gruppen definiert sind,
(ii) Erwärmung und/oder Infrarotbelichtung der Druckplattenvorstufe, wobei die Beschichtung von hydrophil in hydrophob oder von hydrophob in hydrophil umgewandelt wird und dabei ohne Nassentwicklungszwischenschritt ein lithografischer Druckmaster erzeugt wird, und
(iii)Auftrag von Druckfarbe und/oder Feuchtwasser auf den lithografischen Druckmaster mittels einer lithografischen Druckpresse.

2. Verfahren nach Anspruch 1, **dadurch gekennzeichnet, dass** zumindest eine der VWB-Gruppen eine Isocytosinylgruppe ist.

3. Verfahren nach Anspruch 1 oder 2, **dadurch gekennzeichnet, dass** das Polymer aus VWB-modifizierten Phenolharzen, VWB-modifizierten Poly(meth)acrylaten, VWB-modifizierten Polyestern, VWB-modifizierten Polyethern, VWB-modifizierten Polyurethanen und Gemischen und Copolymeren dergleichen gewählt wird.

4. Verfahren nach Anspruch 3, **dadurch gekennzeichnet, dass** das Polymer ein VWB-modifizierter Polyether ist.

5. Verfahren nach Anspruch 4, **dadurch gekennzeichnet, dass** das Molekulargewicht des VWB-modifizierten Polyethers zwischen 100 g/Mol und 5.000 g/Mol liegt.

6. Verfahren nach einem der Ansprüche 4 oder 5, **dadurch gekennzeichnet, dass** der VWB-modifizierte Polyether ein VWB-modifiziertes Polyethylenoxid, ein VWB-modifiziertes Polypropylenoxid oder ein Gemisch oder Copolymer dergleichen ist.

7. Verfahren nach Anspruch 3, **dadurch gekennzeichnet, dass** das Polymer ein VWB-modifiziertes (Meth)acrylathomopolymer oder (Meth)acrylatcopolymer mit einer Struktureinheit mit einer Isocytosinylgruppe in der Seitenkette ist.

8. Verfahren nach Anspruch 7, **dadurch gekennzeichnet, dass** das Molekulargewicht des VWB-modifizierten (Meth)acrylathomopolymers oder (Meth)acrylatcopolymers zwischen 500 g/Mol und 500.000 g/Mol liegt.

9. Eine Druckplattenvorstufe, die auf einem Träger, der eine hydrophile Oberfläche aufweist oder mit einer hydrophilen Schicht versehen ist, eine Beschichtung mit einem Polyether enthält, der mit zumindest zwei Gruppen, die vier Wasserstoffbrückenbindungen bilden können, modifiziert ist, wobei die Gruppen als "vierfache Wasserstoffbrückenbindungen" oder "VWB"-Gruppen definiert sind.

10. Druckplattenvorstufe nach Anspruch 9, **dadurch gekennzeichnet, dass** die VWB-Gruppe eine Isocytosinylgruppe ist.

11. Druckplattenvorstufe nach Anspruch 9 oder 10, **dadurch gekennzeichnet, dass** das Molekulargewicht des modifizierten Polyethers zwischen 100 g/Mol und 5.000 g/Mol liegt.

12. Druckplattenvorstufe nach Anspruch 11, **dadurch gekennzeichnet, dass** der modifizierte Polyether ein VWB-modifiziertes Polyethylenoxid, ein VWB-modifiziertes Polypropylenoxid oder ein Gemisch aus beidem ist.

## Revendications

1. Un procédé d'impression lithographique comprenant les étapes ci-après:
(i) la mise à disposition d'un précurseur de plaque d'impression lithographique thermosensible comprenant sur un support ayant une surface hydrophile ou étant revêtu d'une couche hydrophile un revêtement contenant un polymère modifié avec au moins deux groupes pouvant former quatre liaisons hydrogène, lesdits groupes étant définis comme « quadruples liaisons hydrogène » ou groupes « QLH »,
(ii) le chauffage et/ou l'exposition à des rayons infrarouges du précurseur de plaque d'impression, si bien que le revêtement est converti d'hydrophile en hydrophobe ou d'hydrophobe en hydrophile et qu'on obtient ainsi une matrice d'impression lithographique sans étape intermédiaire de développement humide, et
(iii) l'encrage et/ou le mouillage de la matrice d'impression lithographique à l'aide d'une presse à imprimer lithographique.

2. Procédé selon la revendication 1, **caractérisé en ce qu'**au moins un des groupes QLH est un groupe isocytosinyle.

3. Procédé selon la revendication 1 ou 2, **caractérisé en ce que** le polymère est choisi parmi des résines phénoliques modifiées par QLH, des poly(méth)acrylates modifiés par QLH, des polyesters modifiés par QLH, des polyéthers modifiés par QLH, des polyuréthanes modifiés par QLH et des mélanges et copolymères de ceux-ci.

4. Procédé selon la revendication 3, **caractérisé en ce que** le polymère est un polyéther modifié par QLH.

5. Procédé selon la revendication 4, **caractérisé en ce que** le poids moléculaire du polyéther modifié par QLH est compris entre 100 g/mole et 5.000 g/mole.

6. Procédé selon l'une quelconque des revendications 4 ou 5, **caractérisé en ce que** le polyéther modifié par QLH est un oxyde de polyéthylène modifié par QLH ou un oxyde de polypropylène modifié par QLH ou un mélange ou un copolymère de ceux-ci.

7. Procédé selon la revendication 3, **caractérisé en ce que** le polymère est un homopolymère ou copolymère de (méth)acrylate modifié par QLH comprenant une unité structurale contenant un groupe isocytosinyle dans la chaîne latérale.

8. Procédé selon la revendication 7, **caractérisé en ce que** l'homopolymère ou copolymère de (méth)acrylate modifié par QLH présente un poids moléculaire compris entre 500 g/mole et 500.000 g/mole.

9. Un précurseur de plaque d'impression comprenant sur un support ayant une surface hydrophile ou étant revêtu d'une couche hydrophile un revêtement contenant un polyéther modifié avec au moins deux groupes pouvant former quatre liaisons hydrogène, lesdits groupes étant définis comme « quadruples liaisons hydrogène » ou groupes « QLH ».

10. Précurseur de plaque d'impression selon la revendication 9, **caractérisé en ce que** le groupe QLH est un groupe isocytosinyle.

11. Précurseur de plaque d'impression selon la revendication 9 ou 10, **caractérisé en ce que** le poids moléculaire du polyéther modifié est compris entre 100 g/mole et 5.000 g/mole.

12. Précurseur de plaque d'impression selon la revendication 11, **caractérisé en ce que** le polyéther modifié est un oxyde de polyéthylène modifié par QLH ou un oxyde de polypropylène modifié par QLH ou un mélange de ceux-ci.
